

## UNITED STATES PATENT OFFICE

ROYSEL J. COWAN AND PHILIP W. MCCOY, OF TOLEDO, OHIO, ASSIGNEES TO SURFACE COMBUSTION CORPORATION, OF TOLEDO, OHIO, A CORPORATION OF NEW YORK

## PROCESS OF CASE HARDENING

No Drawing.

Application filed March 8, 1930. Serial No. 434,445.

This invention relates to improvements in the art of case-hardening metal objects by a gaseous medium more particularly ammonia gas and has for its objects to provide a continuous process of case hardening as distinguished from the usual intermittent or batch type process; to provide a process of case hardening that shall permit more complete utilization of the case-hardening constituent 10 of the gaseous medium, and withal to provide a process which shall give a more uniform case than can be obtained by the batch type process heretofore used.

Surface hardening of metals by ammonia 15 gas is known as "nitriding" and nitriding processes as heretofore conducted are fully set forth in the publication entitled "Nitriding Symposium" being the "Transactions of the American Society for Steel Treating", 20 Vol. XVI, October, 1929, No. 5, published by American Society for Steel Treating, Cleveland, Ohio.

As will clearly appear from the above entitled publication, nitriding as heretofore 25 conducted is a batch type process. That is to say the articles to be nitrided are placed in a suitable container adapted to be placed within a suitable heating chamber without being moved through the chamber and ammonia gas passed through the container during 30 the heating operation. The more usual type of equipment for carrying on the nitriding operation consists of a gas tight box wherein the articles can be supported on a 35 screen, the inlet tube for ammonia gas extending along the bottom of the box below the screen while the outlet is at the front end and near the top of the box. (See page 74 of said publication.) The box type process, however, gives more or less erratic results and it has, therefore, been proposed to provide 40 means such as a fan for agitating or stirring up the nitriding gases in the work container. (See page 150 of said publication.)

The time of nitriding with processes heretofore used varies with the individual method and purpose from 18 to 90 hours and the usual temperature range is from 850 to 1150° F. and the ammonia dissociation is 45 usually kept within 30 to 40 percent.

Now we have discovered and this forms the basis of our invention that nitriding can be carried on at the usual temperatures as a continuous process, that is to say, where the articles are passed in continuous course through 55 a heating chamber, with more uniform results and with a higher degree of dissociation of the ammonia gas and consequently with the use of much less ammonia and in appreciably less time than heretofore, provided the 60 ammonia gas and the work to be nitrided have unidirectional flow as distinguished from counterflow through the heating chamber. As previously stated the usual or permissible limits of ammonia dissociation with prior processes is between 30 to 40 percent. With our process the ammonia dissociation may be practically complete for example 90 percent or more at the outlet from the heating 65 chamber. The heating chamber may be of any suitable form, as for example, a tunnel type muffle chamber provided with suitable means at its ends permitting entry of work into and discharge of work from the heating chamber without inflow of air into the chamber. The work may be moved through the heating chamber in any suitable manner, as for instance, small articles may be placed in wire baskets adapted to be pushed through the heating chamber or a conveyer belt may 70 be provided for supporting the work. The main thing as already stated is that the gas and work shall flow in the same direction. As already indicated the heat-treating temperatures will follow the usual practice. It will, of course, also be understood that the ammonia gas will be introduced into the heating chamber at the work-entering end of the chamber and will leave at the opposite end 75 and that the chamber will contain a plenum of the gas. The gas will, of course, be introduced into the heating chamber under sufficient pressure to cause a flow of the gas 80 through the chamber, the flow being so regulated to obtain as high degree of dissociation 85 at the outlet from the chambers as may be desired.

As already indicated dissociation may proceed to a degree approaching complete disso-

55

60

65

70

75

80

85

90

95

100

2  
ciation at the outlet from the chamber without adversely affecting the results.

What takes place according to our improved process would seem to be substantially as follows: The work while it is being brought up to temperature, is being continually subjected to the action of fresh ammonia gas and consequently the decarburizing action by free hydrogen from dissociated ammonia is prevented, the case hardening taking place progressively with dissociation of the ammonia gas. Our experiments have shown that high dissociation of the ammonia gas will not impair a nitrided case when once formed, but on the contrary actually improves the quality of the case thereby producing a better case in the same length of time than is produced in the intermittent process. It will, therefore, be readily appreciated that according to our invention, the products of dissociation of the ammonia gas are being continually removed from the work by the gas flow and consequently the hydrogen concentration never becomes great enough to exercise any decarburizing effect. However, whatever may be the true explanation of the reaction which takes place by causing the ammonia gas and work to flow in the same direction, the fact remains that our experiments conclusively show that a superior nitrided case can be produced in a shorter time and with less ammonia than by any process heretofore proposed.

Our experiments show that satisfactory results are obtained by introducing all of the ammonia at the charging end of the furnace or muffle but it is within the spirit of the invention to also introduce ammonia at points between the ends of the furnace.

While our improved process has special utility where the case hardening medium is ammonia gas, nevertheless it also has application with other case hardening gases and, therefore, it is not intended to limit the invention except as may be expressed in the appended claims.

What is claimed is:

1. A process of case hardening objects by ammonia gas comprising simultaneously passing said objects and said gas in unidirectional flow through a heating chamber.
2. In a process of case hardening objects where the objects are moving in continuous course through a heating chamber, the step of passing ammonia gas through said chamber in the same direction of flow as said objects.
3. A continuous process of nitriding comprising simultaneously passing the objects to be nitrided and the nitriding gas in unidirectional flow through a heating chamber.
4. A process of nitriding permitting the obtainment of suitable case with ammonia dissociation in excess of 40 percent comprising passing the objects through a heating

chamber and simultaneously passing ammonia gas through said chamber in the same direction of flow as said objects.

5. A process of nitriding permitting obtainment of suitable case with ammonia dissociation approaching complete dissociation comprising passing the objects through a heating chamber and introducing into said chamber for flow in the same direction as said objects a regulated stream of ammonia gas.

In testimony whereof we affix our signatures.

ROYSEL J. COWAN.  
PHILIP WM. McCOY.

70

75

80

85

90

95

100

105

110

115

120

125

130